

May 13, 1969

J. E. ROBERTS

3,444,010

FLUID-MOLD CASTING SLAG

Filed Oct. 3, 1966



FIG. 1



FIG. 2



FIG. 3

INVENTOR  
JAMES EARL ROBERTS

BY

*M. L. Pinel*  
ATTORNEY

# United States Patent Office

3,444,010

Patented May 13, 1969

1

3,444,010

## FLUID-MOLD CASTING SLAG

James E. Roberts, Huntington, W. Va., assignor to The International Nickel Company, Inc., New York, N.Y., a corporation of Delaware

Filed Oct. 3, 1966, Ser. No. 583,911  
Int. Cl. C23c 1/12

U.S. Cl. 148—22

5 Claims

The present invention is directed to an improvement 10 in the fluid-mold casting process to produce ingot castings made of nickel and nickel-containing alloys having improved surface and improved metallurgical quality and to a special casting slag composition for use in such a process.

The fluid-mold casting process has now been available to the art for a number of years and has been employed successfully in connection with the production of ingot castings made of a number of different metals. In accordance with the process, a quantity of molten slag is placed 20 at the bottom of an ingot mold and molten metal conditioned for the production of an ingot is teemed into the mold through the slag. During teeming, the slag advances upward on the surface of the metal and forms a thin coating on the ingot mold surface. The coating remains 25 during the casting process and separates the ingot from the ingot mold. When conditions in respect of metal and slag temperature, melting point and composition of the metal and the slag are compatible, an ingot is produced having a greatly improved surface 30 as compared to that obtained when no casting slag is employed. The initial work conducted in accordance with the fluid-mold casting process involved the use of silicate type slags. These slags operated successfully in conjunction with the casting of metals such as mild steel and stainless steel. However, when it was attempted to use the silicate type slags with nickel and nickel-base alloys, it was found that numerous difficulties were encountered. Thus, with many alloys, an intolerable pick-up of silicon 35 in the ingot resulting from interaction between the molten metal and molten slag was encountered, yielding ingots which did not meet chemical specifications. In addition, defects were encountered in the surface of many ingots which have been classified as "notch" defect, a peripheral indentation about the ingot toward the toe portion and as "shotted-surface" defect, which apparently involves emulsification of slag and metal and is usually most evident toward the top of the ingot. These defects required extensive and expensive overhaul of the ingots before 40 further mill processing could be successfully undertaken. The result has been that the advantages contemplated through the use of the fluid-mold slag casting process, namely, improved ingot yield and better ingot surface, were not obtained in many instances. A further development in relation to slag chemistry involved the deletion 45 of silica as a slag constituent and the use of a titania-calcium oxide-alumina type slag to provide an improved fluid-mold casting composition for use with nickel-containing alloys, particularly of the age hardening types. Further experience with this slag material has demonstrated that even further improvement was necessary. For 50 example, it was found that in the fluid-mold casting of nickel ingots intended for the production of wrought nickel products for electronic uses, an intolerable pick-up of titanium from the slag was encountered. This resulted in ingots which were chemically out of definition and which were not acceptable. Furthermore, it was found that while in many instances highly satisfactory ingot surfaces were obtained in the production of nickel and nickel 55 alloy ingots with the improved slag, that in other instances unsatisfactory ingot surfaces, e.g., shotted surface, were 60 still obtained.

2

I have now discovered an improved casting slag composition and process for fluid-mold casting of nickel, nickel-base and nickel containing alloys which provides improved ingot surfaces and greater recovery of metal from the ingot into hot rolled products.

It is an object of the present invention to provide an improved fluid-mold casting slag particularly useful for the production of ingots made of nickel and nickel-containing alloys.

Another object of the invention is to provide a fluid-mold casting process applicable to nickel and nickel-containing alloys which provides improved ingot surface and improved metal yield upon hot rolling of the ingots, as well as improved metallurgical quality.

Other objects and advantages of the invention will become apparent from the following description taken in conjunction with the accompanying drawing in which:

FIGURE 1 is a reproduction of a photograph depicting the surface of a 20 inch square by 90 inch long nickel ingot produced in accordance with the concepts of the present invention.

FIGURE 2 is a reproduction of a photograph depicting the surface of a 20 inch square by 90 inch long nickel-chromium-iron alloy ingot produced in accordance with the invention, and

FIGURE 3 is a reproduction of a photograph of a hot rolled billet produced from an age hardenable nickel-chromium alloy ingot cast in accordance with the invention which was hot rolled without any surface overhauling.

Generally speaking, the present invention is directed to a casting slag composition consisting essentially of, by weight, about 20% to about 40% alumina, about 25% to about 50% calcium oxide, with the alumina content not exceeding the calcium oxide content by more than 5 weight percent, about 5% to about 20% magnesium oxide, about 3% to about 10% sodium oxide, and about 10% to about 30% of an alkaline earth fluoride ingredient from the group consisting of cryolite ( $Na_3AlF_6$ ), potassium aluminum fluoride ( $K_3AlF_6$ ) and fluorspar ( $CaF_2$ ). Advantageously, the casting slag composition contains about 35% to about 50% calcium oxide, about 25% to about 40% alumina, about 5% to about 15% magnesia, about 10% to about 30% of an alkaline earth fluoride from the group consisting of cryolite, potassium aluminum fluoride, calcium fluoride and about 3% to about 10% sodium oxide. A preferred slag composition contains about 35% to about 40% calcium oxide, about 25% to about 40% alumina, about 5% to about 8% magnesia, about 10% to about 20% cryolite, about 5% to about 10% fluorspar and about 3% to about 6% sodium oxide. The slags produced in accordance with the invention have a flow point on heating in the temperature range of about 2300° F. to about 2450° F. The special slag compositions are essentially devoid of silica and titania, although, in some instances, for example, those in which minor pick-up of silicon is permissible, up to about 3% silica may be present. Titania should not exceed about 0.5%, by weight, e.g., 0.1% or 0.2%. Metal oxides such as manganese oxide, chromium oxide, nickel oxide and copper oxide are preferably absent but may be in some cases present in amounts up to about 1% each. Impurities harmful to nickel and nickel alloys, including arsenic, lead, tin, zinc, sulfur, etc., should be absent from the slag. For purposes of controlling the flow point on heating the slag to be in the advantageous neighborhood of 2300° F. to about 2450° F. in the case of nickel and nickel-containing alloys, including nickel-chromium, nickel-chromium-iron, nickel-copper alloys, cupronickel alloys, etc., the ingredients for forming the slag are carefully proportioned. The bulk of the slag composition com-

prises calcium oxide and alumina with the alumina being present in amounts not exceeding the calcium oxide by more than 5 weight percent. Magnesia and sodium oxide in the controlled amounts specified hereinbefore assist in controlling the melting point. Magnesia is employed in amounts not exceeding 20% and preferably not exceeding about 15% since greater amounts undesirably raise the slag melting point. The fluoride ingredients, namely, cryolite, potassium aluminum fluoride and fluorspar, are employed in the amounts described for purposes of further controlling fluidity and melting point of the slag. In compounding the slag, it is important that the dry ingredients be thoroughly blended prior to melting since it is otherwise found impractical to secure a uniform slag composition in the melting procedure. Melting advantageously is conducted in a submerged electrode furnace. A number of satisfactory slag compositions are set forth in the following Table I:

TABLE I

| Slag No. | CaO, percent | Al <sub>2</sub> O <sub>3</sub> , percent | MgO, percent | CaF <sub>2</sub> , percent | Na <sub>2</sub> AlF <sub>6</sub> , percent | K <sub>2</sub> AlF <sub>6</sub> , percent | Na <sub>2</sub> O, percent | Flow point on heating, ° F. |
|----------|--------------|------------------------------------------|--------------|----------------------------|--------------------------------------------|-------------------------------------------|----------------------------|-----------------------------|
| 1-----   | 37           | 37                                       | 6            | 5                          | 10                                         | -----                                     | 5                          | 2,440                       |
| 2-----   | 35           | 35                                       | 6            | 5                          | 14                                         | -----                                     | 5                          | 2,400                       |
| 3-----   | 43           | 27                                       | 10           | 5                          | 10                                         | -----                                     | 5                          | 2,320                       |
| 4-----   | 37           | 37                                       | 6            | -----                      | -----                                      | 15                                        | 5                          | 2,440                       |
| 5-----   | 35           | 35                                       | 10           | -----                      | -----                                      | 15                                        | 5                          | 2,380                       |

The special casting slag composition is particularly advantageous for the production of ingots in commercial wrought nickel containing 99% and more of nickel, nickel-copper alloys containing 50% or more of nickel, cupronickel alloys containing nickel in amounts as low as about 29% and the balance essentially copper, and nickel-chromium-iron alloys containing 30% or more of nickel, up to 50% of iron and up to 30% of chromium. The alloys may also contain other usual alloying ingredients such as up to about 10% molybdenum, up to about 10% columbium, up to about 30% cobalt, up to about 5% tungsten, up to about 5% manganese, up to about 3% silicon, up to about 0.5% carbon, up to about 2% vanadium, up to about 6% aluminum, up to about 6% titanium, up to about 0.2% zirconium, up to about 0.5% magnesium, etc. Stainless steels containing as little as 7% nickel and up to 75% iron may also be treated in accordance with the invention.

Compositions of nickel-containing alloys which may be satisfactorily fluid-mold cast in accordance with the invention are set forth in the following Table II:

TABLE II

| Alloy No. | Percent Ni | Percent C | Percent Mn | Percent Fe | Percent Si | Percent Cu | Percent Cr | Percent Al | Percent Ti         | Percent other |
|-----------|------------|-----------|------------|------------|------------|------------|------------|------------|--------------------|---------------|
| 1-----    | 99.5       | 0.06      | 0.25       | 0.15       | 0.05       | 0.05       | -----      | -----      | -----              | 0.003         |
| 2-----    | 99.5       | 0.09      | 0.18       | 0.05       | 0.03       | 0.03       | -----      | -----      | -----              | -----         |
| 3-----    | 66         | 0.12      | 0.9        | 1.35       | 0.15       | 31.5       | -----      | -----      | -----              | -----         |
| 4-----    | 55         | 0.06      | 0.01       | 0.05       | 0.02       | 44         | -----      | 0.02       | -----              | -----         |
| 5-----    | 65         | 0.15      | 0.6        | 1.0        | 0.15       | 29.5       | -----      | 2.8        | 0.5                | -----         |
| 6-----    | 32         | 0.04      | 0.75       | 46         | 0.35       | 0.30       | 20.5       | -----      | -----              | -----         |
| 7-----    | 32         | 0.04      | 0.75       | 44.5       | 0.35       | 0.15       | 20.5       | -----      | -----              | 1.0           |
| 8-----    | 76.0       | 0.04      | 0.2        | 7.2        | 0.20       | 0.10       | 15.8       | -----      | -----              | -----         |
| 9-----    | 73         | 0.04      | 0.7        | 6.75       | 0.3        | 0.05       | 15         | 0.8        | -----              | 2.5 0.85 Cb   |
| 10-----   | 71         | 0.04      | 2.25       | 7.2        | 0.12       | 0.10       | 16         | -----      | -----              | 3.0           |
| 11-----   | 42.7       | 0.05      | 0.45       | 34.0       | 0.4        | 18.5       | 0.25       | -----      | 2.5 6.2 Mo         | -----         |
| 12-----   | 52.5       | 0.04      | 0.2        | 18.0       | 0.2        | 19.0       | 0.6        | -----      | 0.8 5.2 Cb, 3.0 Mo | -----         |

In order to give those skilled in the art a better understanding of the invention, the following illustrative examples are given:

#### Example I

A melt weighing about 9880 pounds made of a commercially pure nickel alloy containing about 99.5% nickel, about 0.09% carbon, not more than 0.3% manganese, not more than about 0.1% iron, not more than about 0.1% silicon, not more than about 0.1% copper, and not more than about 0.003% titanium was prepared for casting in an induction furnace. A casting slag melt made from a charge of blended dry ingredients containing about 37% calcium oxide, about 37% alumina, about 6% magnesia, about 5% fluorspar, about 10% cryolite and about 5% sodium oxide added as sodium carbonate was pre-

75 without ingot overhauling thereby enabling a yield in-

pared in a submerged electrode furnace and was heated to about 3100° F. 20 inch by 20 inch square ingot molds were set up on copper stools. About 250 pounds of the molten casting slag was poured into the bottom of the first ingot mold. This was sufficient to extend upwards 5 within the ingot mold and cover about 3 inches vertically at the bottom of the mold. Nickel from the induction furnace heat was teemed from a bottom pour ladle at a temperature of about 2870° F. into the ingot mold at a steady rate through the slag pool to completely fill the ingot with metal and flush the excess casting slag from the top of the mold. The remaining ingot molds were then filled in the same manner. Metal from the ingots met the rigid chemical specification for this grade of material. The resulting ingots were inspected and found to have an excellent surface which permitted them to be hot rolled without any surface overhauling. The surface of one of the ingots is depicted in the accompanying FIGURE 1.

#### Example II

An ingot of a nickel-chromium-iron alloy containing about 32% nickel, about 0.04% carbon, about 0.75% manganese, about 0.35% silicon, about 0.3% copper, about 20.5% chromium, and the balance essentially iron, was produced by the fluid-mold process employing a fluid-mold casting slag having the composition set forth in

Example I. When the ingot was stripped from the mold, it was found to have a high quality surface free from the shotting defect. The appearance of the ingot is depicted in the accompanying FIGURE 2. The highly satisfactory result achieved with this material contrasts with the results obtained in fluid-mold casting the alloy using both the silicate type slag and the titania-lime-alumina slag of the prior art. Each of the prior art casting slags resulted in a shotted surface with this alloy. Thus, with the silicate type slag about 75% of ingots produced from this alloy required milling and about 60% of ingots produced in this alloy using the titania-lime-alumina slag required milling. However, the ingots produced with the new fluid-mold casting composition described herein could be hot rolled 70 without ingot overhauling thereby enabling a yield in-

crease at the hot rolled stage on the order of 3% to 5% by weight.

Example III

Ingots made of an age hardenable nickel-chromium alloy containing about 7% iron, about 16% chromium, about 3% titanium, about 0.04% carbon, about 0.15% silicon, and the balance essentially nickel, were produced by the fluid-mold casting process employing a slag having the composition set forth in Example I. The ingots were 18 inches square and 48 inches long. Ingots stripped from the mold demonstrated an excellent surface which permitted hot rolling to bloom without ingot overhaul. The surface of a hot rolled shape having a 10 inch by 15 inch section produced from the 18 inch square ingot of this alloy without ingot overhaul is depicted in the accompanying FIGURE 3. It was found that with this particular alloy the prior fluid-mold casting slags did not produce results any better than those achieved with no slag at all. The ability to produce the high quality ingot surface on this alloy using the special fluid-mold casting slag of the present invention enables a yield increase at the hot rolled stage on the order of about 10% by weight as compared to prior practice.

The special fluid-mold casting slag compositions provided in accordance with the invention must be carefully controlled to secure the desired results. In particular, the alumina content should not exceed the lime content by more than 5 weight percent while maintaining other slag ingredients in the ranges set forth hereinbefore or it becomes impractical to obtain the required melting point even with the use of fluoride ingredients. For example, a slag containing 5 moles of CaO and 3 moles of  $Al_2O_3$  with no other ingredients representing a weight content of 52.5%  $Al_2O_3$ , has a flow point on heating which is far in excess of 2450° F. and remains too sluggish and refractory to produce good nickel alloy ingot surfaces in slag casting even when diluted with a fluoride ingredient such as fluorspar.

Although the present invention has been described in conjunction with preferred embodiments, it is to be understood that modifications and variations may be resorted to without departing from the spirit and scope of the invention as those skilled in the art will readily understand. Such modifications and variations are considered to be within the purview and scope of the invention and appended claims.

I claim:

1. A fluid-mold casting slag composition consisting essentially of, by weight, about 20% to 40% alumina, about 25% to 50% calcium oxide, with the alumina content not exceeding the calcium oxide content by more than 5 weight percent, about 5% to about 20% magnesium oxide, about 3% to about 10% sodium oxide, and about 10% to about 30% of an alkaline earth fluoride.
2. A casting slag in accordance with claim 1 containing about 35% to about 50% calcium oxide, about 25% to about 40% alumina, about 5% to about 15% magnesia, about 3% to about 10% sodium oxide and about 10% to about 30% of an alkaline earth fluoride.
3. A casting slag in accordance with claim 1 containing about 35% to about 40% calcium oxide, about 25% to about 40% alumina, about 5% to about 8% magnesia, about 3% to about 6% sodium oxide, about 10% to about 20% cryolite and about 5% to about 10% fluorspar.
4. A casting slag in accordance with claim 1 containing about 35% to about 43% calcium oxide, about 27% to about 37% alumina, about 6% to about 10% magnesia, about 5% sodium oxide and about 15% to about 19% of a fluoride ingredient from the group consisting of fluorspar, cryolite and potassium aluminum fluoride.
5. A casting slag in accordance with claim 1 containing about 37% calcium oxide, about 37% alumina, about 6% magnesia, about 5% sodium oxide, about 5% calcium fluoride and about 10% cryolite.

References Cited

UNITED STATES PATENTS

|           |         |             |       |           |
|-----------|---------|-------------|-------|-----------|
| 2,493,394 | 1/1950  | Dunn et al. | ----- | 164—133   |
| 2,631,344 | 3/1953  | Kennedy     | ----- | 164—133   |
| 3,214,806 | 11/1965 | Fox et al.  | ----- | 164—133   |
| 3,224,887 | 12/1965 | Fox et al.  | ----- | 106—38.27 |

L. DEWAYNE RUTLEDGE, Primary Examiner.

W. W. STALLARD, Assistant Examiner.

U.S. CL. X.R.

75—82, 93; 106—38.27